

## UNITED STATES PATENT OFFICE

1,955,567

MANUFACTURE OF INTERFELTED  
CELLULOSE FIBER STRANDS

Milton O. Schur and Benjamin G. Hoos, Berlin,  
N. H., assignors to Brown Company, Berlin,  
N. H., a corporation of Maine

No. Drawing. Application December 8, 1930,  
Serial No. 500,868

## 8 Claims. (Cl. 8—20)

The subject of this invention is the manufacture of interfelted cellulose fiber strands, and more particularly the manufacture of such strands from relatively short and inexpensive fibers, such as wood pulp, having optimum physical characteristics, including high tensile strength and stretching ability in both wet and dry condition, coupled with softness and a fuzzy surface.

10 In making strands of the foregoing character, the practice is to roll or to twist a narrow waterlaid ribbon of interfelted cellulose fibers made on machinery of the papermaking type to round form, while the ribbon is in a damp and plastic state. The resulting round body of waterlaid, interfelted fibers retains its form when dried from its plastic state and has surprisingly high tensile strength and ability to withstand stretching. When composed of wood fibers, it is, however, apt 15 to be inferior in its physical characteristics to a roving of similar weight and twist produced in the usual dry way from cotton fiber on textile machinery. While not limited thereto, our invention is thus applicable to great economic advantage in the case of wood pulp strands.

The object of the present invention is to improve the physical characteristics of strands of waterlaid, interfelted cellulose fibers of various origins, such as wood pulp, without introducing 20 thereinto foreign materials, such as sizes or binders, which detract from their softness, fuzziness, and other characteristics making for similarity to textile rovings of cotton fiber. We have discovered that the results desired may be attained 25 to such an extent by mercerizing the strands of interfelted fibers that strands of such character composed of wood pulp may even excel in certain respects textile rovings of cotton fiber of equal weight. In speaking about strands in the specification and in the appended claims, we mean either a single strand or intertwined multiple strands, as our invention is applicable in either case. Our invention is, however, especially useful from a practical standpoint in the manufacture 30 of grocery twine consisting of two or more intertwined strands of interfelted wood fibers, where ability to undergo substantial stretching without rupture is desired, as we have found that the mercerization of such twines results in a product which may have even better stretching 35 ability, both dry and wet, than twines of similar weight, twist, and number of plies, in which the plies consist of cotton fiber rovings made on textile machinery.

The following table shows the effect of mer-

cerizing for different periods of time a twine composed of four intertwined strands of interfelted wood fiber and weighing 0.2745 grams per yard:

|            | Dry     |         | Wet     |         | 60   |
|------------|---------|---------|---------|---------|------|
|            | Tensile | Stretch | Tensile | Stretch |      |
|            | Lbs.    | Percent | Lbs.    | Percent |      |
| Original   | 7.88    | 3.8     | 6.00    | 9.1     | 65   |
| Mercerized | 15 sec. | 7.30    | 7.25    | 9.4     |      |
| Do.        | 2 min.  | 7.50    | 12.0    | 6.85    | 10.6 |
| Do.        | 4 min.  | 8.25    | 12.6    | 7.10    | 12.0 |
| Do.        | 6 min.  | 7.75    | 13.0    | 7.00    | 12.0 |
| Do.        | 15 min. | 7.25    | 13.0    | 7.00    | 13.0 |

when mercerization was continued for longer than 70 15 minutes, the results were only slightly superior to those obtained in 15 minutes. Our 15-minute mercerized product more than bears comparison 75 in its physical characteristics with the usual cotton fiber twines of commerce. In fact, not only did a similar weight and similarly twisted twine composed of four independent strands of cotton fiber made on textile machinery have no better tensile strength, but it had notably inferior 80 stretchability than our 15-minute mercerized product.

In determining the per cent. stretch as given in the foregoing table, the specimens were clamped in a vertical Schopper testing machine 85 of the usual type, but before the lower clamp was tightened, a specimen was given a very slight initial stretch by hanging a 200-gram weight thereon. By subjecting the string to the action of the 200-gram weight, variations due to the 90 personal factor in clamping the specimen were avoided. In other experiments, where a 500-gram weight was used to effect the initial stretching action on the string, the results were practically 95 the same, the per cent. stretch at the breaking point being slightly lower in all cases, as would be expected.

In actual practice, where the damp ribbons of interfelted fibers are rolled or furled into strand form, for instance as they are carried on a Four-drainer wire, and are then accumulated by delivery into so-called spinning pots, such as used in collecting rayon yarns coming from spinning machines, the annular masses or cakes of strand material collected in the pots may be advantageously 100 mercerized in the pots. The walls of the pot are usually perforated, so that while the pot and the contained cake are being spun or rotated, a solution of caustic soda of mercerized strength 105 may be sprayed for the desired period of time 110

- over the inner face of the cake, centrifugal action serving to carry the solution through the mass of strand material to effect a uniform mercerizing action. The cake may then be freed of mercerizing solution by delivering a spray of wash water over its inner surface while it is being spun or rotated along with the pot. The cake may then be dried and the dry strand material may be plied and intertwined with similar mercerized strand material into multi-ply yarn or string. It is thus seen that after mercerization, nothing is done to the yarn or strand material to destroy the softness, fuzziness and other qualities imparted thereto by mercerization. 80
15. We are aware of the fact that the mercerization of cotton yarn made on textile machinery has long been known, but the discovery that marked benefits may be realized by mercerizing strands of waterlaid, interfelted fibers of the type 20 of wood pulp is a surprise, especially when one pauses to reflect that cellulose fibers, in being interfelted or laid as ribbons from aqueous suspension and in being rolled or twisted in damp condition to strands, undergo manipulations quite 25 different from those performed by textile machinery on cotton fibers in the production of a roving, and further when one considers that wood fibers under the microscope show a different physical structure and are shorter than cotton fibers. 30
30. In fact, as is well known in the art, wood pulps are invariably of an average fiber length below about 2 millimeters. Again, one might suppose that fine strands of waterlaid, interfelted fibers of relatively short length, such as wood pulp, 35 would disintegrate or soften up to a pulp, especially when subjected to the action of an aqueous swelling agent, such as a solution of caustic soda of mercerizing strength. 100
40. An important advantage of our invention resides in the fact that it makes possible the production of yarns or twines while employing high speed machines of the papermaking type and relatively inexpensive short fibered raw materials, such as wood pulp, the resulting yarns or twines 45 being of a quality comparing favorably with the far more expensive yarns and twines made from cotton fiber on textile machinery. 110
- What we claim is:
1. As an article of manufacture, strand material consisting of interfelted, waterlaid cellulose fibers in mercerized condition and possessing the softness, fuzziness, and other qualities imparted thereto by mercerization. 115
50. 2. As an article of manufacture, a twine consisting of at least two intertwined strands of interfelted, waterlaid cellulose fibers in mercerized condition and possessing the softness, fuzziness, and other qualities imparted thereto by mercerization. 85
3. As an article of manufacture, strand material consisting of a rounded ribbon of interfelted wood fibers in mercerized condition and possessing the softness, fuzziness, and other qualities imparted thereto by mercerization. 85
4. As an article of manufacture, a twine consisting of at least two strands of intertwined, rounded ribbons of interfelted wood fibers in mercerized condition and possessing the softness, 90 fuzziness, and other qualities imparted thereto by mercerization. 90
5. A process which comprises treating strand material consisting of a rounded ribbon of interfelted, waterlaid cellulose fibers with a mercerizing liquor, and washing the liquor from such material and then drying it while preserving therein the softness, fuzziness, and other qualities imparted thereto by mercerization. 95
6. A process which comprises treating a twine consisting of at least two rounded ribbons of interfelted wood fibers with a mercerizing liquor, and washing the liquor from such material and then drying it while preserving therein the softness, fuzziness, and other qualities imparted thereto 100 by mercerization. 105
7. A process which comprises spraying mercerizing liquor over the inner surface of an annular mass of strand material consisting of at least one rounded ribbon of interfelted, waterlaid cellulose fibers while the mass is being spun or rotated in a spinning pot whose walls are perforated, then spraying wash water over the inner surface of the mass while it is thus being spun, and drying the mass. 110
8. A process which comprises spraying mercerizing liquor over the inner surface of an annular mass of strand material consisting of a rounded ribbon of interfelted, waterlaid cellulose fibers while the mass is being spun or rotated in a spinning pot whose walls are perforated, then spraying wash water over the inner surface of the mass while it is thus being spun, drying the washed mass, and plying and intertwisting the dry strand material with similar strand material into multi- 120 ply yarn or string. 125

MILTON O. SCHUR.  
BENJAMIN G. HOOS.